

## 1

3,157,496

## MAGNESIUM BASE ALLOY CONTAINING SMALL AMOUNTS OF RARE EARTH METAL

George S. Foerster, Midland, Mich., assignor to The Dow Chemical Company, Midland, Mich., a corporation of Delaware

No Drawing. Continuation of application Ser. No. 78,318, Dec. 27, 1960. This application Sept. 13, 1962, Ser. No. 223,526

11 Claims. (Cl. 75—168)

This invention relates to a magnesium-base alloy containing at least 85 weight percent of magnesium and is more particularly concerned with a thorium-free magnesium alloy having primarily the following composition:

| Alloying constituent: | Weight percent, | balance Mg |
|-----------------------|-----------------|------------|
| Rare earth metal      | 0.05 to 2       |            |
| Zinc                  | 0.05 to 0.5     | 20         |

The alloy of the invention exhibits excellent high temperature properties comparable to the thorium-containing alloys but avoids the use of expensive thorium metal. The alloy also exhibits good resistance to creep both at ambient room temperature and at elevated temperatures such as 400° F.

The rare earth metals suitable for use in preparing the present alloy are: cerium, lanthanum, praseodymium, neodymium, didymium (a mixture of rare earth metals having praseodymium and neodymium as major constituents) or misch metal (a mixture of rare earth metals). Any of the foregoing rare earth metals may be used alone or in any combination in compounding the alloy. A commercially available misch metal, sometimes called cerium misch metal, containing from 35 to 80 percent of cerium, the balance being rare earth metals and up to 5 percent of non-rare earth metal, is the preferred rare earth metal ingredient of the alloy because of availability, although the use of didymium permits the obtaining of somewhat higher strength properties at given rare earth metal concentrations.

The alloy may be further improved by the addition of from 0.2 to 2 percent by weight of manganese as a matrix strengthening component. If desired, a small amount of zirconium, e.g., not more than about 0.2 percent, may be beneficially employed concurrently with manganese for its grain refining action, although when substantially larger amounts of zirconium are added, there is a tendency for zirconium and manganese to precipitate from the alloy together.

If desired, small amounts of one or more other matrix strengthening components which are well known in the magnesium art may be added to the alloy provided they are compatible therewith, i.e., do not precipitate components therefrom during alloy preparation or otherwise adversely effect high temperature properties of the alloy. However, it is preferred that the alloy of the invention contain at least 95 percent by weight of magnesium.

## 2

The composition is further limited to alloys in which the proportion of zinc is in the range of from 1 to  $\frac{1}{3}$  part of zinc per part of rare earth metal in compositions containing up to about 0.6 percent of rare earth metal, and the proportion of zinc is in the range of from 0.2 to 0.5 percent by weight in compositions containing from about 0.6 to 2 percent of rare earth metal.

While higher physical strength properties are generally obtainable at higher cost upon employing higher proportions of rare earth metal, it is usually to be desired for economic reasons that smaller proportions of rare earth metal be used. Thus, a desirable range of proportions of the present alloy is at least 95 percent of magnesium, from 0.2 to 1 percent of rare earth metal and from 0.067 to 0.5 percent of zinc.

The most preferred proportions of the alloying components in the present alloy are, by weight, from 0.2 to 0.5 percent of rare earth metal and from 0.067 to 0.5 percent of zinc. The most preferred weight ratio of rare earth metal to zinc is about 2 parts of rare earth metal per part of zinc. The most preferred proportion of matrix strengthening component is by weight from 0.5 to 1 percent of manganese.

The alloy may be made in the desired proportions according to the invention by melting together the alloying ingredients in proper proportions or by using "hardeners" of magnesium alloys containing the alloy constituents. Protection from oxidation during alloying is effected by the use of a magnesium chloride-free saline flux as in conventional alloying. The molten alloy may be flux refined by stirring the alloy with additional flux. The so-refined alloy is allowed to settle and then is separated from the flux as by decanting into a suitable casting mold, e.g., a slab mold for rolling stock.

## EXAMPLES

To illustrate the advantageous results which can be achieved by the present invention, a series of compositions according to the invention were prepared and cast into respective rolling slabs (e.g., 2 inches x 4 inches x 8 inches). Each slab was treated as follows: The faces of the slab were scalped to remove surface impurities or inclusions. The slab was heated to about 900° F. and rolled into sheet form. Test coupons were cut from the so-prepared sheet and subjected to physical testing. Compressive yield strength and tensile strength tests were carried out in the longitudinal direction of rolling. The alloy compositions, test conditions and the static strength properties are listed in Table I.

By way of comparison, magnesium-rare earth metal alloys containing, respectively, no zinc, and zinc in rare earth metal to zinc ratios outside the scope of the present invention were prepared and rolled into sheet form and similarly tested. The results of these comparison tests are listed in Table I.

By examination of the data in Table I, it may be seen that the alloy of the invention exhibits better high temperature strength properties and greatly increased creep resistance at elevated temperatures.

Table I

| Test No.   | Composition <sup>1</sup> , Percent by Weight |      | Sheet Preparation (Temper) <sup>2</sup> | Physical Properties |           |     |            | Creep Resistance at 5,000 p.s.i. for 100 hrs., Percent Creep | Temp., °F                                |  |  |
|------------|----------------------------------------------|------|-----------------------------------------|---------------------|-----------|-----|------------|--------------------------------------------------------------|------------------------------------------|--|--|
|            | MM                                           | Zn   |                                         | %E                  | At 75° F. |     | At 300° F. |                                                              |                                          |  |  |
|            |                                              |      |                                         |                     | TYS       | CYS | TS         | TYS                                                          |                                          |  |  |
| 1          | 0.2                                          | 0.1  | -O-                                     | 18                  | 16        | 12  | 31         | 12                                                           | 0.09                                     |  |  |
| 2          | 0.2                                          | 0.2  | -O-                                     | 20                  | 15        | 12  | 31         | 13                                                           | 0.09                                     |  |  |
| 3          | 0.4                                          | 0.2  | -O-                                     | 22                  | 17        | 12  | 32         | 14                                                           | 0.06                                     |  |  |
| 4          | 0.6                                          | 0.4  | -O-                                     | 22                  | 19        | 14  | 33         | 15                                                           | 0.08                                     |  |  |
| 5          | 0.8                                          | 0.4  | -O-                                     | 22                  | 19        | 14  | 33         | 15                                                           | 0.05                                     |  |  |
| Comparison | 0.6                                          | 0.1  | -O-                                     | 22                  | 20        | 12  | 32         | 13                                                           | 1.8                                      |  |  |
| Do.        | 0.2                                          | -O-  | 18                                      | 16                  | 11        | 32  | 11         | 2.5                                                          | 400                                      |  |  |
| 6          | 0.2                                          | 0.1  | -H24                                    | 12                  | 22        | 21  | 33         | 19                                                           | 0.09 (at 8,000 p.s.i.)                   |  |  |
| 7          | 0.2                                          | 0.2  | -H24                                    | 12                  | 25        | 23  | 36         | 21                                                           | 0.26 (at 8,000 p.s.i.)                   |  |  |
| Comparison | 0.2                                          | -H24 | 15                                      | 23                  | 20        | 31  | 18         | Ran away after 70 hours                                      | 400                                      |  |  |
| Do.        | 0.2                                          | 0.4  | -H26                                    | 10                  | 26        | 27  | 36         | 11                                                           | 3.9                                      |  |  |
| Do.        | 0.2                                          | 0.8  | -H26                                    | 12                  | 26        | 28  | 38         | 11                                                           | 5.8                                      |  |  |
| Do.        | 0.2                                          | 1.3  | -H26                                    | 18                  | 24        | 25  | 36         | 12                                                           | Ran away after 1 hour under 6,000 p.s.i. |  |  |

<sup>1</sup> Balance magnesium.<sup>2</sup> -H24 Rolling slab reduced 92% by hot rolling at 850° F., then reduced 30% in one pass at 750° F., (450° F. exit), and heat treated 1 hour at 500° F. MM=Cerium misch metal.

-O=Same as -H24 except terminal heat treatment is at 700° F. instead of 500° F.

-H26=Rolling slab reduced 94% by hot rolling at 800° F., then reduced 35% in one pass at 450° F. (320° F. exit), and heat treated 1 hour at 275° F.

%E=Percent elongation.

TYS=Tensile yield strength in 1,000's of p.s.i.

CYS=Compression yield strength in 1,000's of p.s.i.

TS=Ultimate tensile strength in 1,000's of p.s.i.

Ran away=Creep extension v. time curve became very steep so that the extension could not be measured.

Table II

| Test No. | Composition, <sup>1</sup> percent by Weight |     |     | Creep Resistance at 5,000 p.s.i. load at 400° F. for 100 hours, percent creep | 35 | Test Temp. | Physical Properties of Sheet, Strengths in 1,000's of p.s.i. |     |     |    |
|----------|---------------------------------------------|-----|-----|-------------------------------------------------------------------------------|----|------------|--------------------------------------------------------------|-----|-----|----|
|          | MM                                          | Zn  | Mn  |                                                                               |    |            | %E                                                           | TYS | CYS | TS |
| 8        | 0.4                                         | 0.2 | 0.5 | 0.11                                                                          |    |            |                                                              |     |     |    |
| 9        | 0.3                                         | 0.3 | 0.5 | 0.28                                                                          |    |            |                                                              |     |     |    |
| 10       | 0.4                                         | 0.4 | 1.0 | 0.28                                                                          | 40 | 75° F.     | 4                                                            | 37  | 27  | 42 |
|          |                                             |     |     |                                                                               |    | 600° F.    | 45                                                           | 11  | 18  | 68 |
|          |                                             |     |     |                                                                               |    |            | 2                                                            | 39  | 38  | 46 |
|          |                                             |     |     |                                                                               |    |            | 5                                                            |     |     | 12 |

See footnotes, bottom of Table I.

Additional compositions according to the invention, containing manganese in addition to zinc and rare earth metal, were prepared and cast into rolling slabs. Each rolling slab was reduced 92 percent (in thickness) by hot rolling at 850° F., then reduced 30 percent in one pass at 750° F. (450° F. exit), and heat treated 1 hour at 700° F. Test coupons cut from the so-prepared sheet were tested for resistance to creep at 400° F. In Table II are listed the compositions tested and the percent extension in 100 hours.

Still an additional composition according to the invention containing, by weight, from 0.4 percent of manganese and 0.09 percent of zirconium in addition to 1.3 percent of didymium and 0.3 percent of zinc and the balance commercial magnesium, was prepared and cast into rolling slabs each 2 inches x 4 inches x 8 inches. Each slab was scalped to remove surface impurities or inclusions, heated to about 900° F. and reduced in thickness to about 0.1 inch sheet by rolling. During the rolling operation, the partially reduced slab was occasionally reheated to prevent it cracking on being rolled. The sheet was heat treated at about 1000° F. for an hour, quenched, and cold rolled 1-2 percent per pass through steam heated rolls for a total reduction in the range of 15 to 50 percent. The cold rolled sheet was then heat treated at about 500° F. for an hour. Test coupons were cut from the so-prepared sheet and subjected to physical testing in the longitudinal direction of rolling. The results of tests conducted at both 75° F. and 600° F. are listed in Table III.

Table III

| Test Temp. | Physical Properties of Sheet, Strengths in 1,000's of p.s.i. |     |                                                    |    |
|------------|--------------------------------------------------------------|-----|----------------------------------------------------|----|
|            | Cold Rolled 15% and Heat Treated 1 Hour at 500° F.           |     | Cold Rolled 50% and Heat Treated 1 Hour at 500° F. |    |
|            | %E                                                           | TYS | CYS                                                | TS |
| 75° F.     | 4                                                            | 37  | 27                                                 | 42 |
| 600° F.    | 45                                                           | 11  | 18                                                 | 68 |
|            | 2                                                            | 39  | 38                                                 | 46 |
|            | 5                                                            |     |                                                    | 12 |

Among the advantages of the alloy of the invention is good weldability without stress relief.

This application is a continuation of my copending application, Serial No. 78,318, filed December 27, 1960.

I claim:

1. The improvement in thorium-free magnesium base alloys consisting essentially of a rare earth metal content in the range of 0.05 to 2 percent by weight and a zinc content in the range of 0.05 to 0.5 percent by weight, and the balance magnesium which consists in: maintaining the proportion of zinc in the range from 1 to 1/3 part of zinc per part of rare earth metal in compositions containing up to about 0.6 percent by weight of rare earth metal and the proportion of zinc being in the range of from 0.2 to 0.5 percent by weight in compositions containing from about 0.6 to 2 percent by weight of rare earth metal.
2. The improvement in thorium-free magnesium base alloys consisting essentially of from 0.05 to 2 percent by weight of rare earth metal, from 0.05 to 0.5 percent by weight of zinc, from 0.2 to 2 percent by weight of manganese, not more than 0.2 percent by weight of zirconium, and the balance magnesium which consists in: maintaining the proportion of zinc in the range of from 1 to 1/3 part of zinc per part of rare earth metal in compositions containing up to about 0.6 percent by weight of rare earth metal, and the proportion of zinc being in the range of from 0.2 to 0.5 percent by weight in compositions containing from about 0.6 to 2 percent by weight of rare earth metal.
3. The improvement in thorium-free magnesium base alloys consisting essentially of up to 0.5 percent by weight

of zinc, and having a rare earth metal content in the range of 0.2 to 1 percent by weight, and the balance magnesium which consists in:

maintaining the proportion of zinc at about 1 part of zinc per 2 parts of rare earth metal.

4. The improvement in thorium-free magnesium base alloys consisting essentially of from 0.2 to 1 percent by weight of rare earth metal, from 0.067 to 0.5 percent by weight of zinc, from 0.5 to 1 percent by weight of manganese, not more than 0.2 percent by weight of zirconium, and the balance magnesium which consists in:

maintaining the proportion of zinc in the range of from 1 to  $\frac{1}{2}$  part of zinc per part of rare earth metal in compositions containing up to about 0.6 percent by weight of rare earth metal, and the proportion of zinc being in the range of from 0.2 to 0.5 percent by weight in compositions containing from about 0.6 to 1 percent by weight of rare earth metal.

5. The improvement in thorium-free magnesium base alloys consisting essentially of rare earth metal in the range of 0.2 to 0.5 percent by weight, a zinc content in the range of 0.067 to 0.5 percent by weight, and the balance magnesium which consists in:

maintaining the proportion of zinc in the range of from 1 to  $\frac{1}{2}$  part of zinc per part of rare earth metal.

6. The improvement in thorium-free magnesium base alloys consisting essentially of up to about 0.25 percent by weight of zinc, and having a rare earth metal content in the range of 0.2 to 0.5 percent by weight, and the balance magnesium which consists in:

maintaining the proportion of zinc at about 1 part of zinc per 2 parts of rare earth metal.

7. The improvement in thorium-free magnesium base alloys consisting essentially of from 0.2 to 0.5 percent by weight of rare earth metal, from 0.067 to 0.5 percent by weight of zinc, from 0.5 to 1 percent of manganese,

not more than 0.2 percent by weight of zirconium, and the balance magnesium which consists in:

maintaining the proportion of zinc in the range of about 1 to  $\frac{1}{2}$  part of zinc per part of rare earth metal.

5. 8. A magnesium base alloy consisting essentially of: from 0.2 to 0.5 percent by weight of rare earth metal, zinc in the proportion of about 1 part of zinc per 2 parts of the rare earth metal and the balance magnesium.

9. A magnesium base alloy consisting essentially of: from 0.2 to 0.5 percent by weight of rare earth metal, zinc in the proportion of about 1 part per 2 parts of the rare earth metal, about 0.5 percent by weight of manganese, not more than 0.2 percent by weight of zirconium and the balance magnesium.

10. A magnesium base alloy consisting essentially of: from 0.2 to 0.8 percent by weight of rare earth metal, from 0.1 to 0.4 percent by weight of zinc, and the balance magnesium, the proportion of zinc being in the range of 1 to  $\frac{1}{2}$  part of zinc per part of rare earth metal.

15. 11. A magnesium base alloy consisting essentially of: from 0.2 to 0.8 percent by weight of rare earth metal, from 0.1 to 0.4 percent by weight of zinc, from 0.5 to 0.1 percent by weight of manganese, up to 0.2 percent by weight of zirconium, and the balance magnesium, the proportion of zinc being in the range of 1 to  $\frac{1}{2}$  part of zinc per part of rare earth metal.

References Cited in the file of this patent

UNITED STATES PATENTS

30. 2,420,293 Beck et al. ----- May 13, 1947

FOREIGN PATENTS

513,627 Great Britain ----- Oct. 18, 1939

532,143 Great Britain ----- Jan. 17, 1941

806,104 Great Britain ----- Dec. 17, 1958

115,813 Australia ----- Sept. 17, 1942